

Patented Dec. 4, 1928.

1,693,716

# UNITED STATES PATENT OFFICE.

WILLIAM HOFFMAN KOBBE, OF NEW YORK, N. Y., ASSIGNOR TO TEXAS GULF SULPHUR COMPANY, OF BAY CITY, TEXAS, A CORPORATION OF TEXAS.

## PLASTER BOARD AND THE LIKE.

No Drawing.

Application filed March 14, 1927. Serial No. 175,432.

This invention relates to articles made of hardened plaster and covered in part at least with fibrous material, such as plaster board and the like. The invention contemplates 5 certain improvements in the manufacture of such articles, as well as a new and improved article of this character.

The ordinary plaster boards of commerce are made up of a body of hardened plaster, 10 usually gypsum plaster, covered in whole or in part with fibrous material, usually a wood pulp paper. In accordance with my present invention the fibrous covering of plaster board and similar products is impregnated 15 to a desired extent with sulfur, and preferably the sulfur impregnation is conducted so as to strengthen the bond between the plaster body and its fibrous covering by congealed sulfur. The impregnation of the 20 fibrous covering may advantageously be effected by immersing the plaster board or similar article in a bath of molten sulfur and subsequently permitting the molten sulfur to congeal in the interstices of the fibrous 25 material.

The body or interior of plaster board is ordinarily hardened gypsum plaster. By gypsum I mean calcium sulfate, with or without water of crystallization, plaster of Paris, 30 anhydrite, alabaster and all natural and commercial forms of these substances. Gypsum usually occurs with two molecules of water of crystallization ( $\text{CaSO}_4 \cdot 2\text{H}_2\text{O}$ ) and is calcined until the water of crystallization is reduced to one-half molecule ( $\text{CaSO}_4 \cdot 1/2\text{H}_2\text{O}$ ) 35 or until all of the water of crystallization has been driven off. After calcining and grinding the gypsum is mixed with water which causes it to set or harden. Although the 40 exact chemical changes which take place are obscure, it is probable that the gypsum reverts to its native or initial state with two molecules of water of crystallization. However this may be, so far as the present invention is concerned it is applicable to all 45 forms of set or hardened gypsum plaster regardless of the water content.

Various commercial forms of gypsum or plaster board may be employed in the practice of the invention, such, for example, as rock lath, sheet rock, gyp lap, Sackett board, etc. It is to be understood, however, that the invention is not limited to these products, 50 but may be advantageously applied to any 55 article made up of a hardened plaster body

covered in part at least with fibrous material. The fibrous material may be various pulp and paper products, fabrics, textiles as well as inorganic fibrous materials such as asbestos, fibrous talc, mineral wool and the like. 60

I am aware that gypsum alone has been treated with molten sulfur in an attempt to impregnate it, but I find that certain difficulties are encountered. The lowest temperature at which sulfur may be used is above the calcining temperature of gypsum and therefore the water of crystallization is driven off and the mass of gypsum becomes wholly or in part calcined and weakened. For this reason efforts have been made to 70 modify the melting point of sulfur which is a difficult and impractical thing to accomplish, and attempts have been made to inject sulfur into the gypsum by means of a solvent which is likewise extremely difficult and 75 which, if accomplished, would give very different results from using molten sulfur as a saturating medium.

I have discovered that a sheet of set or hardened gypsum or similar plaster product 80 which is held together and bound with a uniform covering material such as fibre board, may be readily impregnated by immersion in a bath of molten sulfur at 120° to 140° C. without any deleterious results and a preferred embodiment of the process may be 85 described as follows:

Sheets of rock lath, for example, of any appropriate thickness, are cut to size and immersed in a bath of molten sulfur at 120° 90 to 140° C. either in a horizontal or vertical position until the fibre covering has become fully saturated with the molten sulfur together with the surface of the gypsum that is in immediate contact with this fibre covering. This is accomplished in one or two hours or even less, depending upon the thickness 95 of the fibre covering, moisture content and particularly the degree of sulfur penetration desired.

Upon removal from the treating bath the molten sulfur is held within the fibre covering and in the gypsum immediately adjacent thereto by capillarity and this sulfur, due to its low latent heat, very quickly solidifies especially if placed in a current of air or otherwise chilled and the loss from exudation or dripping is negligible. 100

These treated fibre gypsum products if not 105 perfectly flat may be pressed while still hot 110

or after the first solidification of the sulfur and while it is in its monoclinic stage and more or less plastic, and in this way a perfectly true and flat product assured. As a rule, however, the products mentioned are generally flat and this is unnecessary. On the other hand, they may be deliberately curved or otherwise shaped to a slight degree if this is desirable, but it is important to manipulate them while the sulfur is either molten or in its transition stage as one of the great advantages of the treatment is the fixation which is brought about by stable, rhombic crystals of sulfur.

15 In my co-pending patent applications, Serial No. 61,831, filed October 10, 1925, and Serial No. 124,784, filed July 24, 1926, methods are described for coloring sulfur and for coloring various materials with colored sulfur 20 and I find that the processes there described are applicable in the practice of the present invention. In accordance with the methods there described, I may include in the practice of the present invention sulfur soluble dyes 25 with the sulfur and thereby impart attractive shades of color to these fiber gypsum products, and I find that the color penetrates as far as the sulfur itself, and is of a highly permanent nature.

30 Products made in accordance with the invention have numerous practical commercial advantages. Set gypsum, in itself, or the various products composed in part of set gypsum, is not proof against weather or moisture 35 and consequently cannot be used out of doors. These products are hydroscopic and rapidly disintegrate when exposed to moisture and are readily acted upon by various acids and chemical fumes. They also lack physical 40 strength for many purposes.

45 Plaster board and similar products when treated in accordance with the method of the invention are proof against all normal weather conditions and satisfactorily withstand various acids and chemical fumes. The 50 sulfur saturated fibrous covering, regardless of the degree of penetration of the sulfur into the gypsum itself, entirely protects the enclosed gypsum from any destructive influences, in addition to greatly increasing its strength. By partially impregnating the gypsum as well as the fibrous container or covering, these qualities are enhanced and a 55 product results which is waterproof and acid resistant to a high degree.

The increase in strength under tension, compression and cross-bending amounts to three or four fold and sometimes more, depending to some degree upon the extent of penetration of the sulfur in the underlying 60 gypsum, but very desirable qualities are brought about by treating the fibrous covering only and I am thereby able to produce an acid proof siding and interior roofing material for industrial plants, outdoor advertising signs and billboards, counter and table tops and large waterproof sheets to serve as forms for placing concrete, together with a multitude of other products.

65 The new plaster board product of the invention may be painted, varnished, laquered or shellacked, and will take practically any finish, or it may be colored as hereinbefore described and given a high finish by sanding, 70 buffing polishing. In many cases in order to reduce flammability, it is desirable to give the impregnated article a finishing coat of 75 paint or lacquer. These highly finished materials are suited for radio panels, wall tile and various sanitary products such as parts 80 for partitions, baseboards and as a general substitute for slate and other slab materials.

85 While I have mentioned various commercial forms of gypsum or plaster board, I do not wish to confine myself to these products, 90 since the invention is not limited to these particular products, but is applicable to any form of hardened plaster or gypsum which is covered in whole or in part by fibrous material. The impregnation with sulfur of such products 95 or articles will principally extend to the fibrous material and will generally only affect the plaster which is immediately adjacent to the fibrous material, thereby, however, strengthening the bond between the plaster 100 and its fibrous covering.

I claim:

1. A composition board comprising an interior including hardened plaster covered in part at least by fibrous material, the fibrous material being bonded to the interior of the board by crystals of sulfur.

2. An article of manufacture comprising an interior including hardened plaster covered in part at least by a sulfur impregnated 100 fibrous material, said impregnated material being bonded to the interior of the board by crystals of sulfur.

In testimony whereof I affix my signature.

WILLIAM HOFFMAN KOBBÉ.